

March 10, 1931.

C. C. VAN VOORHIS

1,795,746

BASING CEMENT

Original Filed Feb. 16, 1922



INVENTOR  
Cletus C. Van Voorhis

BY

ATTORNEY

## UNITED STATES PATENT OFFICE

CLETUS CLINTON VAN VOORHIS, OF KINGSTON, NEW JERSEY, ASSIGNOR TO WESTINGHOUSE LAMP COMPANY, A CORPORATION OF PENNSYLVANIA

## BASING CEMENT

Original application filed February 16, 1922, Serial No. 536,942. Patent No. 1,614,506, dated January 18, 1927. Divided and this application filed November 23, 1926. Serial No. 150,232.

This invention relates to cementitious composition and more particularly to a cement for uniting a lamp bulb or the like to a base and is a division of my application Ser. No. 536,942, filed Feb. 16, 1922, relating to electrical devices, which issued Jan. 18, 1927, as Patent No. 1,614,506.

Gas lamps, especially those having a filling of neon gas, find considerable use for ornamental purposes or for sign lighting, and are particularly advantageous when used as small indicating or pilot lamps. These lamps employ a relatively low current and, when they are operated on commercial circuits, it is desirable to provide a resistance in series with each lamp for the purpose of preventing the passage of excessive currents therethrough. The stabilizing resistances frequently employed consist of separate units 20 disposed in the line or of a separate resistance element of such character as to be contained either in the interior of the lamp or in the base thereof. My invention concerns itself with improving this part of the lamp.

One of the objects of my invention is to provide a basing cement having incorporated therewith an electrical conductive material to serve as a stabilizing resistance element which may constitute an integral part of a lamp.

Another object of my invention is the provision of an element which will serve a double purpose, namely, that of a stabilizing resistance or electrical conductive element and as an adhesive medium for securing one portion of a lamp to another.

A further object is the provision of an adhesive cement containing a conductive material for use as a bonding medium to unite a bulb to a lamp base.

The above objects may be accomplished by providing a resistance or conductive material having an adhesive property necessary to a cement and capable of serving to unite the base of the lamp to the bulb. It is common, in the art of manufacturing electric lamps, to secure the base or screw cap to the bulb or envelope in which the source of light is disposed by an interposed layer of cement. 45 This cement which is termed a basing ce-

ment, is usually of a suitable consistency to permit its flow into the base. In practice, the base and bulb are properly juxtaposed until the cement is pressed against the surface of the bulb and the inner surface of the base, after which the cement is hardened by baking, thus bonding the base and the bulb.

In practicing my invention, I employ a suitable basing cement and combine therewith a conductive material in sufficient proportions to provide a given resistance, the necessary adhesive property and the plasticity of the cement, previous to baking, being maintained.

By the provision of a resistance element 55 incorporated in the cement, considerable advantage is derived, inasmuch as the necessity for external resistance devices is avoided and no appreciable amount of space is required 60 for my resistance element when incorporated 70 in a lamp.

The accompanying drawing illustrates an embodiment of my invention as applied to 75 a lamp, part of the structure being shown in section.

The lamp (partly illustrated) may be of any desired type having an envelope 2 containing a filling of a suitable gas and provided with leading-in wires 3 and 4 which extend from, and are sealed in, a pressed 80 portion 6 of the envelope. The leading-in wires conduct current to electrodes (not shown) disposed within the envelope. The electrodes may be of any suitable form, depending upon the use to be made of the lamp.

A hollow threaded member or base 7 is provided and, in lamps of the ordinary type, this base is secured to the envelope by an adhesive medium or basing cement, and one of the leading-in wires of the lamp is connected 85 to the base, the other leading-in wire being connected to an external contact member 8 which is insulated from the shell or body of the base by a separator 9 made of glass or other insulating material.

A lamp constructed according to my invention may be provided with a cement constituting a combined electrically conductive substance as a resistance and an adhesive substance 10 which cement as a whole may be 100

termed a resistance element. An end 11 of the leading-in wire 4 projects from the envelope 2 a sufficient distance to permit a portion and, consequently a given area of the 5 wire, to make contact with the resistance element 10. The leading-in wire 3 extends through the resistance element and the base 7 and is soldered, or otherwise secured to the contact member 8.

10 As illustrated in the accompanying drawing, a portion of the leading-in wire 3 extends through the resistance element or cement 10, which construction necessitates the provision of a layer of insulating material 12 to prevent short-circuiting of the current. Such insulation may be of any desired material and may be applied by the most convenient method. It has, however, been found desirable to employ any suitable insulating 20 varnish or a viscous water solution of sodium silicate which may be applied to the leading-in wire by means of a brush.

When this coating is dry, the layer 12, thus formed, furnishes an efficient insulation. 25 In order to more positively prevent any current from passing through the base adjacent to the end of the leading-in wire 3, a layer 14 of any suitable material as, for instance, glass-wool, asbestos-fiber or the like may be disposed between the end of the base 7 and the resistance element 10. Thus, the contact 30 8 is more perfectly insulated from the resistance element.

When the invention, as above set forth, is applied to a lamp of well known form, in which a so-called flare seal is employed, there will be, instead of the press 6, as illustrated, a space between the resistance element 10 and the envelope which may be filled with 35 glass-wool or insulating material. This will prevent the resistance element, when in a plastic state, from flowing in contact with leading-in wires.

In practice, the required portion of the 40 leading-in wire 3 is given a coating of the insulating material 12. A predetermined amount of plastic cement, containing the proper proportion of conductive material, is then deposited in a base which is slipped over the end of an envelope or bulb, the leading-in wire 3 being, at the same time, threaded through an aperture in the contact element 8 from which it slightly projects. The cement is then hardened by the usual baking 45

process, after which the end of the leading-in wire 3 is soldered to the contact element 8. When the base containing the cement is applied to the bulb, it is obvious that the leading-in wire 4 which projects from the 50 bulb will be disposed within the cement, consequently when the cement hardens, a firm contact is secured between the wire and the cement or resistance element 10.

It will be appreciated that the resistance of 55 the cement or resistance element 10 will de-

pend upon several factors, i. e., the diameter and length of the portion of the wire which makes contact with the element, the dimension of the base and the conductivity of the cement or resistance element. The latter 70

factor is dependent upon the materials used to make a cement conductive and the relative amount of these conductive materials used. The composition which I have found to answer all the requirements preferably consists of a mixture of a suitable filler as, for instance, barium sulphate or marble flour, or both, and a soluble gum such as shellac or bakelite to which is added a suitable conductive substance, such as a metallic powder, 80 as, for instance, a molybdenum or tungsten powder or powdered carbon; to this mixture may be added a suitable solvent, such as alcohol, in sufficient proportion to produce a plastic composition of the desired viscosity.

85 In order to ensure a resistance of about 5000 ohms, using a standard candelabra base, having leading-in wires 4 of 25 mil wire,  $\frac{1}{4}$  inch of one of the wires being in contact with the cement, a cement of the following 90 composition may be used:

|                                                   |                     |
|---------------------------------------------------|---------------------|
| Barium sulphate                                   | 3 parts (by weight) |
| Marble flour                                      | 8 parts             |
| Powdered graphite (pulverized electrode graphite) | 3 parts             |

95 The ingredients are intimately mixed and are made sufficiently plastic and adhesive by means of approximately 5 parts of a shellac 100 solution. The barium sulphate, marble flour and powdered graphite are preferably fine enough to pass through a 60-mesh screen. The shellac solution may be prepared by dissolving one pound of powdered bleached shellac in one quart of methyl alcohol or ethyl alcohol denatured with methyl alcohol.

105 Although I have obtained good results by the use of a shellac solution, it will be evident that, if desirable, the shellac may be mixed with the conductive substance and the filler, a suitable volatile solvent being added to this mixture to produce a plastic composition of appropriate viscosity. When a cement of relatively high temperature resistance is required, bakelite may be substituted for shellac, but, if a cheaper product is desired, Albertol may be employed as the substitute.

110 The ingredients are intimately mixed until their consistency is such as to enable the composition to be readily poured or shaped into any desirable form, after which it may be baked until the solvent is volatilized and a relatively rigid tenacious product is obtained.

115 It will thus be evident that I may prepare the composition of any workable consistency which will permit the composition to be poured and disposed in a given relation to one or more of the component parts of a device 120 which may be secured together by the com- 130

position. Electrical conductors may be suitably disposed or embedded in the composition while in its plastic state and thus secured therein when the composition has become hardened by baking.

By the use of my invention, it is possible to manufacture glow lamps of very small size including a stabilizing resistance, and considerable advantage is thereby obtained. When 10 it is desirable to employ a lamp having a small base, it is obvious that the desired results may be had by my comparatively simple construction and that a small lamp may be placed in a commercial line without expensive 15 additions in the way of stabilizing resistance devices other than the self contained resistance element within the lamp.

The composition, when prepared in accordance with the above directions, is light in 20 weight, has a high temperature resistance, does not crack in drying and possesses, in a high degree, all the desired properties of a cement and a resistance element.

Since my invention may be embodied in 25 many other forms than that shown and described, I do not wish to be restricted to the exact form shown but intend to cover all modifications which lie within the scope of the appended claims.

30 What is claimed is:

1. A basing cement consisting of a volatile solvent, an alcohol soluble gum, a conductive substance, barium sulphate and marble flour.
2. A basing cement consisting of a volatile solvent, barium sulphate, marble flour, carbon and shellac.
3. A composition of matter consisting of the following substances substantially in proportion by weight indicated: barium sulphate 40 3 parts, marble flour 8 parts, powdered graphite 3 parts and a volatile solvent in suitable proportion to produce a plastic mixture.
4. A composition of matter consisting of 45 the following substances substantially in proportion by weight indicated: barium sulphate 3 parts, marble flour 8 parts, powdered graphite 3 parts and a shellac solution 5 parts, the said solution consisting of one 50 pound of shellac dissolved in 1 quart of methyl alcohol.

In testimony whereof, I have hereunto subscribed my name this 20th day of Nov., 1926.

CLETUS CLINTON VAN VOORHIS.

55

60

65